

Patented May 4, 1926.

1,583,549

# UNITED STATES PATENT OFFICE.

ALFRED GEORGE COOPER GWYER AND HENRY WILFRED LEWIS PHILLIPS, OF LONDON, ENGLAND, ASSIGNEES TO THE BRITISH ALUMINUM COMPANY, LIMITED, OF LONDON, ENGLAND.

## METHOD OF TREATING ALUMINUM-SILICON ALLOYS.

No Drawing.

Application filed June 9, 1925. Serial No. 36,043.

To all whom it may concern:

Be it known that we, ALFRED GEORGE COOPER GWYER, a subject of the King of Great Britain and Ireland, and HENRY WILFRED LEWIS PHILLIPS, a subject of the King of Great Britain and Ireland, and both residing at 109 Queen Victoria Street, London, E. C. 4, England, have invented certain new and useful Improvements Relating to Methods of Treating Aluminum-Silicon Alloys, of which the following is a specification.

This invention relates to the improvement of the structure of alloys and especially those containing aluminum.

The object of the invention is to provide improved or alternative methods of and means for improving the physical structure and properties of alloys and especially of aluminum alloys.

In alloys containing aluminum and silicon, the silicon, if present to the extent of about 11 to 15 per cent, may exist in the form of more or less large crystals, or it may be widely dispersed in the eutectic, while in alloys with less than about 11 per cent silicon the silicon is in either case all in the eutectic, though again its dispersion may vary between very wide limits, the degree of dispersion being, of course, greatest in the completely "modified" and least in the completely "normal" alloys. The greater dispersion is accompanied by improved physical properties in the alloy.

We have made a large number of experiments in connection with the improvement of the structure of alloys and have found as the result of our investigations that the mechanism of the process known as "modification" is such that the phenomena concerned are not solely and exclusively characteristic of a particular series of alloys but the process of "modification" is capable of being applied and extended to a large number of or many alloy systems.

We have formulated a theory which we now put forward to assist in the understanding of our invention as we find it useful to that end, whether indeed it includes the true explanation of what happens or not.

According to this theory we assume that certain alloys when in the molten state and above a certain temperature consist of homogeneous liquids of which the constituent

metals are in a state of molecular dispersion (i. e., true solution), but that below a certain temperature which is probably not much above the freezing point the molecules become associated in groups of colloidal particles. With ordinary rates of solidification the colloidal groups are allowed sufficient time to coalesce into aggregates of microscopic dimensions with the result that "normal" structures ensue, but with ultra-rapid rates of solidification the tendency is for the colloidal state to persist after solidification, in which case the resultant structures cease to be normal and approximate to "modified."

Such an ultra-rapid rate of cooling may be produced, say by quenching from the molten state in iced brine. In actual practice it is not usually possible to chill in this manner nor, generally speaking, in any other manner with a degree of rapidity sufficiently great to obtain "modified" structures, especially in the case of sand castings, but recourse must be had to some suitable "modifying" agent and in our view the true function of such a "modifying" agent is that of a "colloid protector" and the process of "modification" consists simply in the more or less complete stabilization of the colloidal state.

Whether this be the true explanation or not is immaterial but it assists in understanding and in predicting.

Thus on our theory it follows that the best results will only be obtained in practice if the correct quantity of "modifying" agent, or "colloid protector", be employed and experience has proved that this is the case.

This can be illustrated by adding progressively increased quantities of a "modifying" agent to a previously "normal" alloy, whence it is seen that the structure is improved up to a certain percentage addition but after that deterioration or "reversion" sets in.

We have also found by a series of hardness determinations according to the Brinell method that accompanying the structural change there is a marked improvement in the mechanical properties and these experiments also emphasize the desirability of employing the "colloid protector" in the correct amount.

What happens in the case of one series of

alloys is not necessarily a guide to the behaviour of another series because to take a specific example, aluminum-iron alloys behave differently from aluminum-silicon alloys although they might be expected to be substantially similar. Sodium chloride will "normalize" a "modified" aluminum-silicon alloy. Sodium hydroxide will "modify" a "normal" alloy but sodium hydroxide will "normalize" a "modified" aluminum-iron alloy and sodium chloride must be used for "modifying" the "normal" alloy.

The invention consists in a process for physically varying the structure of aluminum-silicon alloys which comprises the addition to the molten alloy of a peroxide of an alkali metal, for example sodium peroxide.

The invention also consists in the methods of "modifying" alloys hereinafter described.

The invention further consists in improved or "modified" alloys prepared according to the process described herein.

In carrying the invention into effect in one form applied by way of example to an aluminum-silicon alloy containing 87 per cent aluminum and 13 per cent silicon, we introduce a small percentage, say for complete conversion about 3 per cent by weight, of sodium peroxide into the molten alloy preferably in small portions at a time because the reaction is strongly exothermic. The sodium peroxide is forced to the bottom of the melt which need not be raised higher in temperature than is usual in aluminum foundry practice. The melt is then vigorously stirred; a strong reaction takes place and the melt rises in temperature with each addition. After skimming off the dross and slag and cooling to the temperature desired for pouring the metal is poured in the usual way, preferably in a chill mould. In the case of alloys which are already partially "modified" or partially "reverted" smaller percentages of "modifying" agent may be employed and this should preferably be done.

In place of peroxide of sodium peroxide of potassium or other alkali metal peroxide or mixtures of such peroxides may be used.

The proportion of "modifying" agent may be varied, an experiment readily showing the best quantity to employ. Our experiments have shown that in the case of an aluminum-silicon alloy containing a medium amount of silicon, namely 11 per cent, the Brinell hardness number increased by about 8 to 9 per cent as the quantity of "modifier" was increased from nothing to about 3 to 5 per cent and then decreased so that when the addition was as high as  $7\frac{1}{2}$

per cent there was a marked reduction in the Brinell number. It is better to make other tests as well as the Brinell test according to the usual methods of testing alloys but the Brinell number gives a fair indication.

"Modification" or structural change brings with it a marked improvement in the mechanical properties.

The invention is not limited to treatment of the above alloys as long as the alloys are largely predominant in aluminum and contain silicon as the other principal ingredient whether there are also appreciable amounts of other elements of aluminum and silicon or not.

Further, the proportions given above are not limiting proportions.

The alloys to be "modified" should not contain more than a small percentage of iron and should not be held long in the molten condition after the addition so that, for example, the operation of casting should be carried out either in chill moulds or in sand moulds provided with suitable chills so as to accelerate the rate of solidification of the metal in the heavier portions of the casting.

Having now described our invention what we claim as new and desire to secure by Letters Patent is:—

1. A method for physically varying the structure of alloys largely predominant in aluminum and containing silicon as the other principal ingredient which consists in the addition to the molten alloy of a peroxide of an alkali metal.

2. A method for physically varying the structure of alloys largely predominant in aluminum and containing silicon as the other principal ingredient which consists in the addition to the molten alloy of sodium peroxide.

3. A method for physically varying the structure of alloys largely predominant in aluminum and containing silicon as the other principal ingredient which consists in the introduction into the molten alloy at a temperature only slightly above the melting point of the alloy of a peroxide of an alkali metal.

4. A method for physically varying the structure of alloys largely predominant in aluminum and containing silicon as the other principal ingredient which consists in the introduction into the molten alloy at a temperature only slightly above the melting point of the alloy of sodium peroxide.

In testimony whereof we have signed our names to this specification.

ALFRED GEORGE COOPER Gwyer.  
HENRY WILFRED LEWIS PHILLIPS.